

## UNITED STATES PATENT OFFICE

2,656,329

## SYNTHETIC FIBER PREPARATION

George E. Ham, Decatur, Ala., assignor to The Chemstrand Corporation, Decatur, Ala., a corporation of Delaware

No Drawing. Application October 15, 1952,  
Serial No. 314,951

6 Claims. (Cl. 260—30.6)

1

This invention relates to a new method of preparing synthetic fibers from copolymers of acrylonitrile. More particularly the invention relates to a new solvent for acrylonitrile polymers, and to completely miscible mixtures including acrylonitrile copolymers, from which mixtures quality fibers can be extruded.

This application is a continuation-in-part of my copending application Serial No. 117,506, filed September 23, 1949, for "Synthetic Fiber Preparation," now abandoned.

It is well-known that copolymers of over 75 percent acrylonitrile are capable of being fabricated into high strength fibers. The conventional technique for preparing fibers from these copolymers involves the dissolution of the copolymer in a suitable solvent and thereafter extruding the viscous solution so prepared through an orifice into a medium which removes the solvent and precipitates the acrylonitrile copolymer in a continuous form. Many solvents have been proposed but many of them are impracticable due to the cost and due to the tendency of the solution to gel upon standing, especially at elevated temperatures encountered in the spinning operation.

The primary purpose of this invention is to provide a new low cost solvent for the preparation of synthetic fibers. A further purpose of this invention is to provide a solvent which forms more stable mixtures or solutions of acrylonitrile copolymers. A still further purpose of the invention is to provide a method of forming fibers of high tensile strength and desirable elongation.

It has been found that mixtures of diethyl phosphite and N,N-dimethylacetamide or N,N-dimethylformamide are excellent solvents for acrylonitrile copolymers. Not all copolymers of acrylonitrile are soluble in all mixtures of diethyl phosphite and the said N,N-dimethylamides. It has been found, however, that there is a definite relationship between proportions of diethyl phosphite and the N,N-dimethylformamide or N,N-dimethylacetamide and the quantity of acrylonitrile in the copolymer. However, it has been found that solvent mixtures containing more than 30 percent of diethyl phosphite will not dissolve polyacrylonitrile and copolymers of more than a fixed maximum amount of acrylonitrile. The maximum acrylonitrile content may be defined by the relationship  $y=90+0.14x$ , wherein  $x$  is the percent of the N,N-dimethylamide and  $y$  is the maximum acrylonitrile proportion in the copolymer. In addition, it has been further found that polymers containing

more than 90 percent by weight of acrylonitrile are insoluble in pure diethyl phosphite while polymers containing 90 percent or less of acrylonitrile are soluble in pure diethyl phosphite. In order to dissolve the polymers containing more than 90 percent by weight of acrylonitrile, it is preferred to employ at least 30 percent diethyl phosphite in the solvent mixture. It has been found that solvent mixtures containing 1 to 70 percent of N,N-dimethylamide and 30 to 99 percent diethyl phosphite will dissolve polymers containing more than 90 percent by weight of acrylonitrile and are useful in the practice of the present invention.

Suitable acrylonitrile copolymers which may be dissolved in mixtures of diethyl phosphite and the N,N-dimethylamides are the copolymers of more than 90 percent by weight of acrylonitrile and at least 0.2 percent of another polymerizable monomer, for example vinyl acetate and other vinyl esters of monocarboxylic acids, methyl methacrylate and other alkyl esters of methacrylic acid, ethyl acrylate and other alkyl esters of acrylic acid, methacrylonitrile, vinylidene chloride, ethyl maleate and other alkyl esters of maleic acid, ethyl fumarate and other alkyl esters of fumaric acid, styrene and other vinyl substituted aromatic compounds, alpha-methyl styrene and other isopropenyl aromatic hydrocarbons, vinyl chloride and other vinyl halides, vinyl pyridine and other vinyl substituted heterocyclic amines, and other polymerizable monomers capable of polymerization with acrylonitrile. The mixture of diethyl phosphite and the N,N-dimethylamide is also a solvent for copolymers of more than 90 percent by weight of acrylonitrile and a plurality of other monomers, for example the copolymers of acrylonitrile, methacrylonitrile and vinyl acetate as described and claimed in copending application Serial No. 786,153, filed November 14, 1947, by Reid G. Fordyce and George E. Ham.

In the practice of this invention, as it is in the preparation of all acrylonitrile fibers, the molecular weight of the polymer is of critical importance. The polymer should have a molecular weight in excess of 10,000 and preferably in excess of 25,000. These molecular weights are determined by measuring the viscosity of the polymer when dissolved in a suitable solvent, such as N,N-dimethylformamide, in the manner well known to the art. It is also very desirable to use acrylonitrile copolymers which are substantially uniform throughout with respect to the chemical composition and physical structure,

Such uniform copolymers enable the practice of the invention more economically, permitting the utilization of continuous uninterrupted spinning and greatly minimizing fiber fractures and clogging of the spinnerets.

In the practice of this invention the polymers of acrylonitrile are used in finely divided form, although massive polymers may be ground to desired particles, preferably solvent-non-solvent polymerization procedures are employed in the preparation of the polymer. The subdivided states of the polymers obtained by spray drying the emulsions, or by filtration and subsequent drying of the solid polymers enable them to be used directly. The finely divided polymer is mixed with the solvent mixture in any type of mixing device, such as a dough mixer or a homogenizer. It is desirable to use a solution of as high a concentration of polymer as possible, but the maximum concentration is dependent upon the molecular weight of the polymer.

To obtain fibers of optimum physical properties polymers of molecular weights in excess of 25,000 are used, and when using such polymers it is only possible to dissolve from five to 35 percent in the solvent mixture without exceeding practicable viscosity values. Although as low as five percent of the polymer can be used in spinning operations, such concentrations are undesirable because they necessitate the removal and recovery of too much solvent from the extruded solution, thereby increasing solvent recovery cost and reducing spinning speeds by reason of the longer periods required for coagulation. The concentration of the polymer in the solution is preferably between seven and 25 percent but will ultimately be determined by considering the desired physical properties of the fiber and the speed of spinning, which speed is a function of the concentration and viscosity of the polymer solution. The viscosity will depend upon the chemical composition and the molecular weight of the polymers. The optimum proportions can best be determined by selecting a uniform molecular weight polymer having good fiber forming properties and dissolving it in the smallest amount of the mixture of diethyl phosphite and either N,N-dimethylformamide or N,N-dimethylacetamide necessary to form a viscous solution capable of extrusion at convenient temperatures.

The fibers are spun by extruding the solution of the acrylonitrile polymer through an orifice, or a spinneret having a plurality of orifices, into a medium which removes the solvent. The volume of the solution passed through the spinneret per unit of time must be constant in order to produce a fiber of uniform size. This is best achieved by using a positively driven gear pump constructed of corrosion resistant metals, such as stainless steel, and adapted to deliver a constant flow of solution regardless of minor changes in viscosity and regardless of the resistance offered by the spinneret. It is also desirable to pass the solution through one or more filters before reaching the spinneret in order to remove all possible traces of foreign matter and particles of incompletely dissolved polymer. The polymer solution may be delivered to the gear pump by means of pressure applied by an inert gas to the liquid surface of the solution reservoir, which must be heated to maintain the solution fluid enough to pass through the conduits. The gear pump, filter devices and conduits to the spinneret are preferably heat insulated and may be

heated to maintain the body of solution in liquid state. The extruding operation should be conducted at elevated temperatures but far enough below the boiling point of the solvent to prevent bubbles or other irregularities in the fiber.

The medium into which the solution is extruded and which removes the solvent may be either liquid or gaseous. The method involving the use of liquids is known as "wet spinning"; and usually utilizes aqueous media, which may have salts or other water soluble compounds dissolved therein. The spin bath may be any liquid which is a non-solvent for the acrylonitrile polymer but which either dissolves the solvent mixture or converts it into a soluble compound. The solvent is leached out of the stream of polymer solution, which first becomes a viscous stream, and finally a solid filament. When a spinneret with a plurality of apertures is used the several streams of polymer converge and ultimately form a single fiber. The spin bath must necessarily be of sufficient size to permit the complete, or substantially complete, removal of the solvent mixture. Obviously, the rapidity of extrusion will affect the size of the spin bath, high speeds requiring much longer baths. The temperature of the bath also affects the size, higher temperatures permitting more rapid diffusion of the solvent mixture from the fiber and enabling the use of shorter baths.

The wet spinning method of fiber preparation is particularly adaptable to the use of mixtures of diethyl phosphite and either N,N-dimethylacetamide or N,N-dimethylformamide as the polymer solvent. Because of the slower rate of solution of the solvent mixture in water as compared to the rate of solution of other known solvents, for example undiluted N,N-dimethylformamide and undiluted N,N-dimethylacetamide, it is possible to obtain clear, transparent fibers, whereas the fibers prepared from solutions in conventional solvents on precipitation in water are cloudy and opaque. For this reason it is frequently desirable to use longer precipitation baths or spinning baths adapted to provide longer immersion periods.

The use of mixtures of diethyl phosphite and the said N,N-dimethylamides as solvents for acrylonitrile copolymers is also adapted to "dry spinning" operations, wherein air, steam, nitrogen or other gas, or mixtures of gases which are inert at the spin temperature, are used to remove the solvent. This method operates at higher temperature; and the solvent mixture is evaporated from the surface of the fiber. The maximum temperature to which the fibers can be subjected is approximately the boiling point of the solvent mixture, since evaporation within the body of the fiber may cause bubbles or other defects. The fiber may be heated by convection from the hot gaseous medium or by radiation from the walls of the spinning cell. Generally a combination of both convection and radiation is involved, but methods involving principally radiation are generally more efficient and permit the operation with the wall temperature considerably in excess of the boiling point of the solvent mixture. The evaporation of the solvent mixture from the fiber surface and the speed of the fiber prevent the development of a temperature exceeding that to which the fiber is stable to decomposition. The dry spinning method is particularly useful at high rates of extrusion.

In general, the methods of both wet and dry

spinning commercially used are adaptable for spinning from solutions in mixtures of diethyl phosphite and N,N-dimethylacetamide or N,N-dimethylformamide, but special considerations may be involved due to the different chemical nature of the solvent mixtures. Automatic machinery for spinning continuously, drying the thread if necessary, and winding it on suitable spools may be modified with the teaching of this specification. As in the case of most synthetic fibers, the fibers of acrylonitrile copolymers spun from the solvent mixture solutions may be stretched to develop optimum physical properties. If desired part of the necessary stretching may be accomplished in the spinning medium by drawing the fiber out of the bath at a rate more rapid than the rate of extrusion.

Further details of the practice of this invention are set forth with respect to the following examples.

*Example I*

A copolymer of 95 percent by weight of acrylonitrile and five percent of vinyl acetate was prepared in an aqueous medium. This polymer was dispersed to the extent of ten percent in a mixture of equal parts of diethyl phosphite and N,N-dimethylacetamide. Upon heating the dispersion to 100° C. a homogeneous solution was obtained which retained its stability when cooled to room temperature.

The same polymer was dispersed in a mixture of 25 percent by weight of N,N-dimethylacetamide and 75 percent diethyl phosphite. The dispersion was heated to 140° C. for a prolonged period but no evidence of solubility was observed.

*Example II*

A copolymer of 99 percent by weight of acrylonitrile and one percent of vinyl acetate was prepared by polymerization in an aqueous medium. The polymer was dispersed in a mixture of 70 parts by weight of N,N-dimethylacetamide and

30 parts of diethyl phosphite. Upon heating the dispersion to 100° C. a transparent solution was obtained, which retained its homogeneity after cooling to room temperature.

5 The same polymer was dispersed in a mixture of equal parts of N,N-dimethylacetamide and diethyl phosphite. The dispersion was heated to 140° C. for a prolonged period but no evidence of solubility was observed.

10 The invention is defined by the following claims.

I claim:

15 1. A fiber-spinning composition comprising a homogeneous miscible mixture of an acrylonitrile copolymer and a liquid dispersion medium consisting of 30 to 99 percent of diethyl phosphite and one to 70 percent of a dimethylamide selected from the group consisting of N,N-dimethylacetamide and N,N-dimethylformamide, the acrylonitrile copolymer being a polymer of more than 90 percent and up to 90+0.14 multiplied by the percentage of dimethylamide in the liquid dispersion medium, by weight of acrylonitrile and at least 0.2 percent of another polymerizable monomer, said copolymer having a molecular weight of at least 10,000.

20 2. A fiber-spinning composition as defined in claim 1 wherein the dimethylamide is N,N-dimethylacetamide.

25 3. A fiber-spinning composition as defined in claim 1 wherein the dimethylamide is N,N-dimethylformamide.

30 4. A fiber-spinning composition as defined in claim 1 wherein the polymerizable monomer is vinyl acetate.

35 5. A fiber-spinning composition as defined in claim 4 wherein the dimethylamide is N,N-dimethylacetamide.

40 6. A fiber-spinning composition as defined in claim 4 wherein the dimethylamide is N,N-dimethylformamide.

GEORGE E. HAM.

No references cited.